

# UNITED STATES PATENT OFFICE.

WILLIAM H. BUELL, OF NEW HAVEN, CONNECTICUT, ASSIGNOR TO WINCHESTER REPEATING ARMS COMPANY, OF NEW HAVEN, CONNECTICUT, A CORPORATION OF CONNECTICUT.

## PRIMING CHARGE.

1,174,669.

Specification of Letters Patent.

Patented Mar. 7, 1916.

No Drawing. Original application filed October 21, 1913, Serial No. 796,441. Divided and this application filed June 18, 1914. Serial No. 845,875.

*To all whom it may concern:*

Be it known that I, WILLIAM H. BUELL, a citizen of the United States, residing at New Haven, in the county of New Haven, State 5 of Connecticut, have invented a new and useful Improvement in Priming Charges; and I do hereby declare the following to be a full, clear, and exact description thereof.

This application is a division of my 10 application which has become Patent No. 1,106,343, issued August 4, 1914.

My invention relates to a priming charge for use in igniting explosives, which is of especial utility in igniting the various 15 smokeless and black powders when used in center fire and rim fire ammunition.

The purpose of my invention is to produce a priming charge which is particularly suited for use with powders as now employed 20 in firearms, and particularly small arms, such charge producing an explosion of not too great local pressure, and of sufficient heat, and leaving substantially no harmful residues; my invention further contemplates 25 the modification of the flash of the priming charge, giving it greater length, and contemplates also the creation of an alkaline residue, which measurably neutralizes the harmful acid residue of the explosion of the 30 powder, particularly of smokeless powder.

According to my invention I produce a priming charge by mixing intimately a detonating salt of hydrazoic acid with a suitable nitrated organic body. For instance, I 35 may add 3 parts by weight of nitro cellulose (preferably high nitrogen insoluble) to 1 part of lead hydrazoate, and mix the same to produce a substantially homogeneous product. While the detonating salts of 40 hydrazoic acid are too brisant for use alone in firearms, and especially in small arms, the mixture above described will be found suitable for such use, the local pressure of the explosion being reduced and its heat increased. Substantially no residue is left 45 which may injure the shell or the bore of the arm. While I prefer to use the lead salt, I may use other detonating salts of hydrazoic acid, for instance the silver salt; I may 50 even use the mercury salt, although this salt does not give all the contemplated advantages, as it leaves a residue which is apt to form a harmful amalgam with the metal of the shell.

In place of the nitro cellulose I may employ some other suitable nitrated organic body such for instance, as nitrated starch, the aromatic nitro compounds as trinitrotoluene; the nitro derivatives for carbamid or urea as nitro urea; the aromatic diazo salts 60 as diazo benzene nitrate; and the aromatic diazo amido compounds as diazo amido benzene. While the proportions most suitable for the mixture may differ with various substances and also with various powders in 65 connection with which the mixture is to be used, they are easily determined by anyone skilled in the art. I desire it to be understood that it is possible that some nitrated organic bodies, in combination with a detonating salt of hydrazoic acid, may not produce a primer having the explosive qualities above described, and that I therefore include in my invention the use of such bodies only 70 as will in such combination produce such a 75 primer.

It is also to be understood that the term "detonating salt" of hydrazoic acid as used in the art, and by me in this specification, refers only to a salt of the heavy metals, and 80 does not include salts of the alkali metals, although such salts may have slight detonating properties under certain abnormal conditions.

My invention further contemplates the 85 presence of a third substance for the purpose of leaving an alkaline residue suited to neutralize wholly or measurably the acid residue left by the burning of the powder, particularly of smokeless powder, and also 90 any acid residue which might be left from the explosion of the other ingredients of the primer. This substance is a salt or other compound which either is not affected by the explosion or is broken up by the explosion, and in either case leaves the residue 95 suitable for the purposes indicated. I may use sodium or potassium carbonate, barium nitrate, or potassium nitrate. I prefer, however, to use an alkali metal salt of hydrazoic 100 acid, or an alkaline earth metal salt, or a double alkali metal and other metal salt, of such acid; such as for instance, the sodium salt, or the potash salt, or the potassium cobalt salt of such acid. The use of these last 105 mentioned substances has the further great advantage of producing an increased flash, in addition to causing the residue of the ex-

losion of the primer to be alkaline. I may for instance mix 6 parts by weight of lead hydrazoate and 11 parts of nitro cellulose (preferably the high nitrogen insoluble) 5 with 3 parts of sodium hydrazoate. It will be found that this mixture when exploded, will have all the advantages above claimed for the mixture of the lead salt and nitro cellulose alone, and will have the additional 10 advantages of an increased flame, and of a beneficial alkaline residue. The proportions may have to be varied under different circumstances and conditions, and with different materials and for different powders, but they can readily be ascertained by anyone skilled in the art. It is possible that some 15 compounds which upon ignition leave an alkaline residue and particularly some members of the group of alkali metal, alkaline 20 earth metal, and double alkali metal and metal salts of hydrazoic acid, may not operate as described in the combinations indicated, and, if so, they are not included in my invention. In my claims I group the above 25 mentioned salts of hydrazoic acid under the general term of alkali metal salts of hydrazoic acid.

The mixtures above specifically referred to, either of two substances, or of three substances, constitute a fine white or light colored mass which may be moistened with a gum solution and then introduced into the primer cups, where it is seated under heavy pressure, and may then, if desired, be covered with paper or foil, or by a thin film of collodion. An anvil of any suitable construction may then be inserted into the cups. When the primer is to be used in rim fire ammunition it is preferably given the treatment with the gum solution and then driven into the annular rim of the cartridge shell by centrifugal force. It may then be covered by collodion.

I have found that I may increase the sensitiveness of the mixture to a high degree, by first mixing the nitrated organic body, as for instance the nitro cellulose, with the alkaline residue producing salt, for instance the sodium hydrazoate, treating the mixture 45 with amyacetate or other suitable solvent, in sufficient amount to obtain the proper consistency, permitting the mixture thus treated to harden and then grinding the same, and then adding to the ground substance the detonating salt, as for instance, lead hydrazoate. Glass may be added at the same time with the detonating salt. By this operation I obtain a primer in which the alkaline residue producing salt is more 50 intimately mixed with the nitrated organic body than would be the case if all three ingredients were simultaneously mixed in a dry state, and the sensitiveness of the mixture is thereby greatly increased. I obtain 55 moreover a further useful result, namely

that the particles of the alkaline residue producing salt are surrounded by a film or covering of the nitrated body, so that such particles are measurably insulated from contact with the metal of the shell, and interaction between the two is measurably prevented. 70

The primer mixtures described in the above specific examples, especially those containing the third ingredient, are homogeneous 75 in character and of the proper igniting quality, so that a hot and uniform flame is produced without excess of local pressure and with a minimum of harmful residue or none at all. The flame produced has the proper velocity and intensity to ignite the powder charge before imparting any appreciable motion to it before ignition, and thus effects an explosion having the maximum pressure near the breech of the gun, and not one 80 which is delayed until the charge nears the muzzle, the portion of the barrel least adapted to withstand bursting pressure.

While I may add other substances to my priming mixture, I prefer not to do so. 85 Thus, chlorate of potash, or some other oxidizing compound, such as the perchlorates, nitrates and peroxids of barium, potassium, etc., may be added to the mixture, or in part substituted for certain ingredients, but their 90 presence is usually undesirable owing to the production of an increased local pressure.

I have also found that a mixture of a detonating salt of hydrazoic acid and an alkali metal salt of such acid forms a priming 100 charge adapted for use in firearms. Such charge may be composed for example, of 45 parts by weight of lead hydrazoate and 55 parts by weight of sodium hydrazoate. In such a charge the brisant effect of the lead 105 salt is toned to a sufficient extent and a maximum value is obtained with regard to alkaline residue.

The alkali metal salt of hydrazoic acid may also be mixed with a suitable non-gaseous fuel and a suitable oxidizing compound to produce a successful priming charge. Such charge may be composed of, for example, 35 parts of sodium hydrazoate, 35 parts of antimony sulfid and 30 parts of potassium 110 chloride. In such a charge the alkali metal salt has for its principal purpose to neutralize measurably the injurious acid residue formed by the reaction between the other ingredients of the charge. The alkali 115 metal hydrazoate, as used in my invention, is of particular value because it is itself explosive and therefore adds this value to the charge in addition to its value in leaving an alkaline residue.

I claim:

1. A priming charge containing a mixture of a detonating salt of hydrazoic acid, a nitrated organic body and a compound which upon ignition will leave an alkaline residue,

- substantially as and for the purpose described.
2. A priming charge containing a mixture of a detonating salt of hydrazoic acid, 5 a nitrated organic body and an alkali salt of hydrazoic acid, substantially as and for the purpose described.
3. A priming charge containing a mixture of a detonating salt of hydrazoic acid, 10 nitro cellulose and an alkali salt of hydrazoic acid, substantially as and for the purpose described.
4. A priming charge containing a mixture of lead hydrazoate, a nitrated organic 15 body and an alkali salt of hydrazoic acid, substantially as and for the purpose described.
5. A priming charge containing a mixture of lead hydrazoate, nitro cellulose and 20 an alkali salt of hydrazoic acid, substantially as and for the purpose described.
6. A priming charge containing a mixture of lead hydrazoate, nitro cellulose and sodium hydrazoate, substantially as and for 25 the purpose described.
7. A priming charge containing a mixture of a detonating salt of hydrazoic acid and a finely divided substance, the particles 30 of which contain a nitrated organic body and an alkali salt of hydrazoic acid, substantially as and for the purpose described.
8. A priming charge containing a mixture of a detonating salt of hydrazoic acid and a finely divided substance the particles 35 of which contain nitro cellulose and an alkali salt of hydrazoic acid, substantially as and for the purpose described.
9. A priming charge containing a mixture of a detonating salt of hydrazoic acid and a finely divided substance the particles 40 of which contain nitro cellulose and sodium hydrazoate, substantially as and for the purpose described.
10. A priming charge containing a mixture of lead hydrazoate and a finely divided 45 substance the particles of which contain nitro cellulose and sodium hydrazoate, substantially as and for the purpose described.
11. A priming charge containing a mixture of a detonating salt of hydrazoic acid 50 and an alkali salt of said acid, substantially as and for the purpose described.
12. A priming charge containing a mixture of a detonating salt of hydrazoic acid and sodium hydrazoate, substantially as and 55 for the purpose described.
13. A priming charge containing a mixture of lead hydrazoate and sodium hydrazoate, substantially as and for the purpose 60 described.
- In testimony whereof I have hereunto set my hand in the presence of two subscribing witnesses.

WILLIAM H. BUELL.

Witnesses:

FRITZ V. BRIESEN,  
JOHN A. FERGUSON.